

R. W. STEARNS.

RESISTANCE MATERIAL.

APPLICATION FILED FEB. 19, 1920.

1,394,949.

Patented Oct. 25, 1921.

252-490



(Ampere) - Volts  
Characteristic Curves for Lamp-Black Concrete



Curing Curves for 18% Lamp-Black Concrete

Inventor:  
Ralph W. Stearns,  
by Alfreds. Danck.  
His Attorney.

X R

# UNITED STATES PATENT OFFICE.

RALPH W. STEARNS, OF SCHENECTADY, NEW YORK, ASSIGNOR TO GENERAL ELECTRIC COMPANY, A CORPORATION OF NEW YORK.

## RESISTANCE MATERIAL.

1,394,949.

Specification of Letters Patent. Patented Oct. 25, 1921.

Application filed February 19, 1920. Serial No. 359,953.

To all whom it may concern:

Be it known that I, RALPH W. STEARNS, a citizen of the United States, residing at Schenectady, in the county of Schenectady, 5 State of New York, have invented certain new and useful Improvements in Resistance Material, of which the following is a specification.

My invention relates to resistance material and has for its object a substantially uniform product with desired electrical characteristics produced in a simple and economical manner.

Specifically, my invention relates to the 10 production of a plastic resistance material having a so-called negative ampere-volt characteristic *i. e.*, a material in which the resistance decreases with an increase of voltage or power input. A material of this character is practically essential to the construction of a protective reactor designed to absorb the energy of high frequency transients in accordance with the disclosures of U. S. 15 patent to Creighton No. 1,317,002. Many materials constructed partly of conducting material and partly of insulating material mixed together so as to have this negative ampere-volt characteristic cannot be produced uniformly in large quantities, or do 20 not possess the characteristic sufficiently pronounced, or are very expensive to manufacture.

By my invention, however, these difficulties are avoided. I have discovered that 25 lampblack added to a non-conducting plastic such as concrete in relatively small percentages, varied to suit the particular characteristic desired, gives a substantially uniform and economical product which is very 30 reliable when cured in the manner more fully set forth hereinafter in detail.

For a more complete understanding of the 35 nature and objects of my invention reference should be had to the following detailed description when taken in connection with the accompanying drawing in which:

Figure 1 shows diagrammatically characteristics to be obtained with varying percentages of lampblack in resistance material 40 made in accordance with my invention; Fig. 2 similarly shows the law by which the percentages of lampblack to be employed may be determined, and Fig. 3 shows diagrammatically the effects of various methods

of curing the resistance material of my invention. 55

The resistance material of my invention has a plastic base of relatively non-conducting material. The material preferably employed is based mainly on cement. A material based on cement which I have found may be employed with advantage has Portland cement and white river sand intimately mixed together in the usual manner substantially in the proportions of 1:2 by volume. 60

To give this material the desired electrical characteristics, I add to this plastic mixture from 17 to 25 per cent. by volume of fine lampblack, and intimately mix this lampblack throughout the mass. The lampblack 70 preferably employed by me is obtained from crude petroleum.

In order to get a uniform product, the resistance material made in this fashion should be cured in ovens in an atmosphere 75 of steam raised to a temperature of between 170° C. and 180° C. at atmospheric pressure. This curing should continue uninterrupted for a period of from 450 to 500 hours after which, as a general rule, the 80 product should be dried out for a period of 48 hours in air at 100° C. As seen from Fig. 3, the quality of the resistance of the material so made is increased in a reliable and uniform manner and at the end of 500 85 hours has reached a practical maximum, which in service lasts substantially indefinitely without change.

Resistance material made in this way for 90 percentages of lampblack varying from 17 to 25 as above described, under the tension of increasing voltages exhibited the so-called negative ampere-volt characteristic, as indicated by the curves drawn in Fig. 1. Here it is seen that the curves for the 95 smaller percentages of lampblack exhibit this characteristic in the more pronounced fashion. Material having about 18% lampblack is for general use in reactors the most serviceable. Lampblack used in percentages in excess of 25% renders the material 100 too conducting to exhibit the negative ampere-volt characteristic to any practical extent, but becomes a stable resistance.

In Fig. 2 I have drawn a curve in which 105 resistance at a given voltage has been plotted against the percentages of lampblack employed in the mixture. From this

it is seen that the conductivity of the resistance material increases substantially in direct proportion to the percentage of lampblack employed.

- 5 While I have here disclosed a specific composition for the resistance material of my invention which is at present the best composition known to me, I would have it understood that this is merely illustrative and  
10 that I do not mean to be limited thereby to the exact composition disclosed, but intend to include recognized equivalents of the ingredients employed in my claims hereunto annexed.  
15 What I claim as new and desire to secure by Letters Patent of the United States, is:  
1. A resistance material comprising a substantially non-conducting base composed mainly of concrete and an admixture of a  
20 relatively small amount of lampblack.  
2. A resistance material comprising a

plastic base composed mainly of concrete, and an admixture of from 17 to 25 per cent. by volume of lampblack dispersed throughout the basic mass.

25

3. A resistance material comprising a plastic base composed mainly of cement and river sand, and an admixture of from 17 to 25 per cent. by volume of petroleum lampblack intimately dispersed throughout 30 the basic mass.

4. A resistance material having a negative ampere-volt characteristic comprising a plastic non-conducting base mainly composed of Portland cement and river sand, 35 and an admixture of a relatively small per cent. by volume of lampblack, the whole being cured until a substantially uniform product results.

In witness whereof, I have hereunto set 40 my hand this 17th day of February, 1920.

RALPH W. STEARNS.